

## UNITED STATES PATENT OFFICE

LINN BRADLEY, OF MONTCLAIR, NEW JERSEY, AND EDWARD P. MCKEEFE, OF PLATTSBURG, NEW YORK, ASSIGNEES TO BRADLEY-MCKEEFE CORPORATION, OF NEW YORK, N. Y., A CORPORATION OF NEW YORK

## PRODUCTION OF CHEMICAL PULP

No Drawing. Application filed September 2, 1926, Serial No. 133,292. Renewed January 23, 1931.

This invention relates to the production of chemical pulp, and to the treatment of residual liquors for the regeneration of cooking liquors.

5 More particularly the invention relates to cyclic and interrelated operations in which two different kinds or types of sulfur-containing cooking liquors are employed, of which soda is the base, some of 10 the same sulfur being present, in one instance, in one type of cooking liquor as a sulfite and being present, in another instance, in another type of cooking liquor as sodium sulfid, and with successive employment of some of the same soda as an active 15 compound in each of the two types of cooking liquors. The two types of cooking liquors may be generally described as an acid sulfite of sodium cooking liquor and as a sodium 20 hydroxide-sodium sulfid cooking liquor. Some of the soda and some of the sulfur may in part be present as other compounds.

Among the particular improvements which 25 the invention presents are operations or steps in which cooking liquor for one type of cooking operation is regenerated (at least in part) from constituents of residual liquor from the other type of cooking operation. The acid sulfite of sodium cooking liquors, to 30 which the invention particularly relates, are those which contain both sodium bisulfite and sulfurous acid when charged into the digester or which contain these ingredients after the introduction of sulfur dioxide into 35 the liquor contained within the digester, for example by relieving sulfur dioxide from one digester into another. The other type of cooking liquors, to which the invention particularly relates, are cooking liquors which 40 contain at least as much sodium hydroxide as sodium sulfid, and usually with the amount of sodium hydroxide considerably in excess of the amount of sodium sulfid.

45 According to one embodiment of the invention, wood chips are cooked with cooking liquor which contains a suitable amount of sodium bisulfite and of sulfurous acid, the resulting residual liquor is separated from the pulp, another lot of wood is cooked with 50 cooking liquor which contains a suitable

amount of sodium hydroxide and a considerable amount of sodium sulfid, the sodium hydroxide being employed in larger amount than the sodium sulfid, the resulting residual liquor is separated from the pulp, and the residual liquors are subjected to concentrating and furnacing steps to form recovered soda products which are employed in the production of further cooking liquor.

55 The residual liquor from the acid cook is 60 advantageously admixed with residual liquor from the alkaline cook, to combine with and fix reactive acid constituents thereof and to form an admixed residual liquor which is either mildly acid, neutral or alkaline to litmus, and the mixing step is regulated for this result. Considerable organic matter usually 65 separates out from solution as a result of such mixing treatment. This liquor is subjected to a concentrating step in any suitable 70 manner. In order to facilitate the subsequent steps of the residual liquor treatment, the mixed liquor may be further treated. For example, the liquor may be subjected to concentration in a suitable multiple-effect evaporator in which the liquor is subjected to rapid and forced circulation adjacent the heating elements so as to prevent, or so as to minimize the effect of, organic 75 deposits thereon, especially in the effects which contain the most highly concentrated liquor. Suitable liquor pumps may be employed in this step for maintaining the rapid and forced circulation. Prior to subjecting the liquor to treatment in the evaporating apparatus, it 80 may advantageously be treated in any suitable manner so as to separate the greater part of the suspended organic matter from the liquor. The separated and somewhat 85 clarified liquor may then be more readily concentrated, and, if desired, a small and regulated amount of a strong reactive sodium compound, e. g. NaOH, may be added to the somewhat clarified liquor so as to redissolve 90 remaining suspended organic matter and thus further prepare the liquor so that it may be 95 readily concentrated in a multiple-effect evaporator, or any other suitable device. The liquor may be sprayed or atomized into hot gases as a part of the concentrating treat- 100

ment, or all of such concentration can be thus effected. The organic matter separated from the liquor prior to concentration thereof may be advantageously returned to the liquor, or to a selected portion thereof, subsequent to the step in which the liquor is subjected to a regulated concentration, for example by returning it to the portion of the concentrated liquor which is to undergo a reducing furnace treatment, or to the portion of the concentrated liquor which is to be treated to form a product containing the soda mainly in the form of sodium carbonate. By adding it to the portion last mentioned, the ratio of organic compounds to sodium-sulfur compounds therein is changed in an advantageous manner.

Any unused portion of residual liquor from the alkaline cook, i. e. that which is not employed for admixing with residual liquor from the acid cook, may be concentrated and constituents thereof subjected to a suitable furnacing treatment whereby a considerable portion of the sulfur content thereof may be driven off from its association with soda, and residuary sulfur is largely present as an oxidized sulfur compound, such as sulfate or sulfite, in the recovered soda product, which contains, as a result of the previous treatment, most of its soda in the form of sodium carbonate, and which is substantially free from sodium sulfid and from sodium thiosulfate. A solution is prepared, which contains the soda thus recovered, and in case there is an amount of sodium sulfid or other sulfur ingredient therein which would prevent or render difficult the production of a suitable cooking liquor for the acid cook of the cycle, by treatment with sulfur dioxide in adequate amount, such solution is subjected to a treatment to remove such material or to change it as may be required. For example, the solution may be subjected to a suitable oxidizing treatment, such as heating it after thoroughly mixing therewith a regulated amount of sodium peroxide; or sodium hypochlorite may be employed as the oxidizing agent, especially when only a small amount of such added reagent is required; or the solution may be subjected to an aerating treatment to remove or oxidize objectionable material. A regulated amount of sodium manganate, or of sodium permanganate, may be employed in such an oxidizing treatment. A moderate amount of lime may be employed subsequently for assisting in the clarification of such oxidized liquor and the clarified liquor separated from the solids. Sodium manganate therefore may be prepared by a suitable furnacing of a mixture of soda and manganese dioxide and such product can be advantageously employed directly without further treatment thereof. Some of the manganese compound required may be obtained by regenerating it from the sediment

removed from the liquor subsequent to the oxidizing treatment, for example prior to adding the lime if any. Some of the sulfid sulfur may even be removed by treating the solution with a regulated amount of sulfate of iron, for example, to form iron sulfid, and a small amount of lime may be added to facilitate in such purification step, and the treated liquor separated from the solids.

The purified solution, which may be prepared in the manner outlined above, is sulfited by means of sulfur dioxide to form cooking liquor of the desired composition which is later employed in a cooking operation of the cycle. The solution may be partially sulfited and the partially sulfited liquor may be further sulfited, for example by absorbing therein sulfur dioxide relieved from a digester. Such further sulfiting may be accomplished either prior to charging the liquor into the digester or subsequent thereto. In all cases, however, sufficient sodium bisulfite and sulfurous acid will be employed in the cooking liquors of the acid type, to perform the required cooking operation.

In carrying out the furnacing operation which produces the soda product which contains mainly sodium carbonate and which is substantially free from sodium sulfid, more air may be employed therein than is required for burning the combustibles obtained from the residual liquor. Thus most of the carbon may be burned and removed, thereby not only aiding in the driving off of sulfur but also minimizing the reducing tendency whereby sodium sulfid might be formed. The excess of air may even reoxidize some  $\text{Na}_2\text{S}$  in case it should be present in objectionable amount.

A regulated portion or all of the admixture of residual liquors, which may be prepared in the manner heretofore described, is subjected to a further treatment, subsequent to the concentrating step described above, whereby constituents thereof are subjected to a heat treatment of a reducing type whereby a soda product is obtained which contains sodium carbonate and sodium sulfid, generally with the sodium carbonate considerably greater in amount than the sodium sulfid but nevertheless containing a relatively large amount of sodium sulfid as compared with the soda product which is to be sulfited to form the acid cooking liquor. This heating operation is advantageously so regulated as to retain in the recovered soda product a considerable portion of the sulfur content of the constituents of the liquor which are thus treated, preferably in the form of sodium sulfid, so that the recovered soda product can advantageously serve as a basis for the production of cooking liquor of the alkaline type of the cycle. Thus the amount of air employed is so regulated that the operation is of a highly reducing nature, and care is taken

to avoid driving off from association with soda, too large an amount of sulfur, and to avoid the formation of an undue amount of sodium sulfate in the recovered soda product. Some sodium sulfite may be present in the product and as a consequence in the cooking liquor produced therefrom, thus modifying the cooking liquor of this type.

When sodium sulfate is added to the cycle 10 to replenish the soda, on account of losses thereof, it is preferably added to the constituents which are to undergo such a reducing furnace treatment, thus forming sodium sulfid therefrom and augmenting that 15 which is otherwise formed.

The sodium carbonate and the sodium sulfid in such recovered soda product are dissolved in water and the solution is subjected to a causticizing treatment with sufficient 20 lime to convert the greater part of the sodium carbonate into sodium hydroxide. In case there is not sufficient sodium hydroxide in the resulting liquor, such compound may be added to or produced therein in any suitable 25 manner. For instance, some sodium carbonate may be added to the liquor which is to be causticized so that liquor of the required composition can be prepared therefrom by a suitable causticizing treatment. The liquid 30 is separated from the lime mud and is employed in a cooking operation of the alkaline type, of the cycle.

In case some of the concentrated mixed 35 residual liquors is to be treated to form a soda product which can serve as a suitable base for the production of the acid cooking liquor, the required portion of such mixed liquors is treated so that constituents thereof are heated and substantially all of the combustibles are 40 burned; at least the heating operation is carried out in such a manner that the resulting soda product contains mainly sodium carbonate and is free from such relatively large amounts of sodium sulfid as are contained 45 in the soda product which is to be causticized to form the alkaline type of cooking liquor. By employing an excess of air, in the manner heretofore stated, a soda product can be obtained thereby which is free from an objectionable amount of sodium sulfid, although 50 it may contain a small amount. Nevertheless, a method has been disclosed above which will permit the production of suitable acid cooking liquor for the cycle of the present invention.

Ordinarily we prefer to so regulate the operations that the amount of alkaline residual liquor produced is adequate to provide a sufficient amount for admixing with the acid residual liquor and a further sufficient amount to provide the soda which serves as the basis for the acid cooking liquor, as this facilitates the production of a soda product which contains mainly sodium carbonate and is substantially free from sodium sulfid, even when

not all of the carbon from organic constituents of the residual liquor is consumed in the furnacing operation. This is especially the case when the alkaline cooking operation has been so carried out that a large portion of the sodium sulfid of such cooking liquor has been caused to react with organic material derived from wood, as such residual liquors appear to very readily part with sulfur when the constituents are heated to the required temperature for a sufficient time.

Residual liquor from the alkaline cook, especially that portion which is to be utilized for producing the high sodium carbonate and low sodium sulfid product, may be employed 50 for a preliminary and partial treating operation such as heating it in contact with wood chips for a sufficient time to cause sodium hydroxide and sodium sulfid, or either or both of them, which may be present in some residual liquor of the alkaline type, to react with the more easily removed constituents of the wood. The treated residual liquor may then be removed to such extent as may be readily withdrawn therefrom, and leaving 55 the residue with the partially treated chips to admix with the main supply of alkaline cooking liquor which is to be subsequently added thereto. The portion of the treated residual liquor which has been removed, may 60 carry a fair amount of suspended organic material, due perhaps to interaction between sodium-organic constituents present in the residual liquor so employed and some of the readily dissolved organic constituents removed from the wood by the partial treatment. However, such suspended organic material is generally of such a fine state of division that it may not be readily separated 65 therefrom, and such liquor may be subjected to the concentrating step with the suspended matter contained therein. Forcing the liquor at high velocity adjacent the heating surfaces of the evaporator may be resorted to so as to facilitate the ready concentration of such 70 liquors. The partially treated chips generally may be properly cooked with a lesser amount of freshly supplied active reagents than where the wood chips have not been given the preliminary partial treatment, and thus effect a further economy since less total 75 chemical is required and a lesser amount of lime may be employed for the causticizing step for preparing cooking liquor. Such treatment of wood chips with alkaline residual liquor presents other advantages, including the ready production of the high sodium carbonate-low sodium sulfid soda product referred to above.

The hot-gases from the furnace, operating 80 under the highly reducing conditions, may carry sulfur dioxide or sulfur trioxide, and may carry some sulfur or some combustible sulfur compounds. The recovery of the sulfur content of the latter may be facilitated 85

by burning such material to  $\text{SO}_2$  or to  $\text{SO}_3$  or a mixture thereof, preferably with the amount of  $\text{SO}_2$  exceeding that of the  $\text{SO}_3$ . This burning step may be carried out in any suitable manner. For example, these hot furnace gases may be admixed with the hot furnace gases from the other type of furnacing operation, if any excess air is therein contained, or a regulated amount of air may be added thereto and the temperature maintained at a sufficiently high point for sufficient time to burn such material to the required point. By suitably regulating such burning operation, the resulting gases may be suitable for generating steam for the cycle, e. g. by passing them through a boiler. These gases generally contain a considerable amount of sodium compound. Passing these gases through an electrical precipitator, preferably at a temperature above the dew point, such solids may be recovered, generally with a high  $\text{Na}_2\text{SO}_4$  content. Such material is advantageously added to that which is to undergo a reducing furnace treatment to form the soda product for the alkaline cooking liquor. Sulfur dioxide may be regained from such gases, when contained therein in amount adequate to justify the step, for example by scrubbing them with a solution which contains sodium carbonate, which may be a solution obtained by dissolving the soda compounds from the product obtained by the furnace treatment which employs an excess of air. Some sodium sulfite may be thus formed in the liquor which is to be employed subsequently in the acid cooking operation. Such sodium carbonate solution is generally purified or freed from sodium sulfid and sodium thiosulfate prior to employing it in such scrubbing step.

The acid cooking liquor may be prepared by first partially sulfiting the liquor and subsequently completing the sulfiting to the required degree. Such sulfur dioxide as is relieved from the digester during or at the end of the cooking operation, for example, may be employed for the completion of the sulfiting of such liquor. The liquor which is charged into the digester generally contains a considerable amount of sodium bisulfite, that is it contains a considerable amount of uncombined  $\text{SO}_2$ . A further amount of  $\text{SO}_2$  may be introduced into the liquor within the digester by any suitable means. For example, some  $\text{SO}_2$  may be liberated from liquor in one digester which may be almost ready to be "blown", into liquor contained in a digester which has considerable time to go before the cooking operation has been completed therein. Thus, instead of relieving  $\text{SO}_2$  into an outside vessel or an absorbing tower, for fortifying the partially sulfited liquor,  $\text{SO}_2$  may be relieved from one digester into another, along with steam, and absorbed in the latter digester. By using a relatively high

content of uncombined  $\text{SO}_2$  in the cooking liquor during the cooking operation, but nevertheless containing a sufficient amount of combined  $\text{SO}_3$ , some advantages are obtained, especially when steam and  $\text{SO}_2$  are relieved from one digester into another.

When sodium carbonate is relied upon for replenishing the soda of the cycle, due to losses, it is preferably added to the liquor which is to be sulfited so as to produce liquor for use in the acid cooking operation. Sulfur required for the operations may be supplied in any suitable manner, for example by burning sulfur in air and absorbing the sulfur dioxide in the liquor or liquors described. When a considerable amount of the sulfur of the cycle is recovered or regained as a sulfite of sodium, the amount of sulfur to be freshly supplied may be reduced accordingly.

The composition of the cooking liquors and the amounts of pulp produced by the two types of cooking liquors, respectively, may vary somewhat; and different kinds of woods may be cooked by either of the cooking liquors. When highly resinous woods, such as certain pines, are cooked by the alkaline liquor and the resulting residual liquor is admixed with the residual liquor from the acid sulfite type of cooking operation of the cycle, for example by cooking gum wood with an acid liquor which contains a fairly high content of combined  $\text{SO}_2$  and a relatively low content of uncombined  $\text{SO}_2$ , the mixing being regulated so as to produce an admixture of residual liquors which is mildly acid, neutral or moderately alkaline to litmus, a considerable amount of organic matter separates out. By separating the liquor from such material, the subsequent steps are improved, viz: the concentration step when multiple-effect evaporators are employed therefor. By regulating the amount of acid liquor added to the alkaline residual liquor, somewhat different grades of products may be separated therefrom, thus the liquor may be added in regulated steps with separation of organic material between the successive additions of liquor. Material suitable for a "soap-stock" may be thus produced.

Somewhat different amounts of the alkaline residual liquor may be admixed with the acid residual liquor. For example, a sufficient amount of acid residual liquor may be admixed with alkaline residual liquor to separate most of the precipitatable organic matter, leaving the mixture slightly acid if desired, then separating the liquor from suspended organic material. The separated liquor, which may still be slightly acid to litmus, may then be treated with a regulated amount of alkaline soda compound to leave the liquor moderately alkaline to litmus. For this result, either some sodium hydroxide may be employed, or some of the sodium carbonate-

sodium sulfid liquor may be added for this purpose, this treatment redissolving small amounts of organic material which may remain in the separated liquor. By regulating 5 the mixing step or steps, described above, a large amount of organic material may be separated and removed from the liquor, and for example by employing only a moderate amount of alkaline compound added there- 10 after, the mixture of the residual liquors may be readily subjected to the concentrating step of the cycle. Instead of employing liquors which contain a suitable alkaline sodium compound which are free from organic matter. 15 for such treatment of the separated and slightly acid mixed liquor, some of the alkaline residual liquor may be thus employed.

By conducting the operations in a manner outlined above, the organic constituents removed from the wood may be made use of for the production of steam for use either in a digester or in a multiple-effect evaporator of the cycle.

When a mixture of steam and  $\text{SO}_2$  is released from a digester, during or at the end or final stage of the digesting operation, and this is not introduced directly into liquor contained in another digester, such mixture of steam and  $\text{SO}_2$  may be utilized by passing it 25 into a hot solution of sodium sulfite or carbonate, for example, contained within a suitable vessel of the closed type, absorbing the  $\text{SO}_2$  therein and permitting steam and uncondensed gases or vapors to pass therefrom 30 in a regulated manner and subsequently employing the steam in another operation of the cycle. For instance, the steam may be permitted to escape from the accumulator under regulated conditions and thence into 35 the steam belt of a multiple-effect evaporator of suitable type and construction, i. e. of suitable acid-resisting material when the steam thus employed contains any constituents of the acid type; or some of the steam may be 40 employed in the heating of a digester charge during the early stages of such heating. Such  $\text{CO}_2$  as the steam may contain may be permitted to escape from the condensed steam in any suitable way. Such sulfite of sodium 45 as is thus formed by reaction between the soda in the liquor within the accumulator and the  $\text{SO}_2$  absorbed from the steam, may be employed in the cooking liquor of the acid type. For example, the liquor may be removed 50 from the accumulator and later subjected to a further regulated sulfiting treatment with suitable vapors or gases which contain  $\text{SO}_2$ , and such sulfiting continued until a cooking liquor is produced which contains 55 the desired amounts and ratio of combined to uncombined  $\text{SO}_2$ . Where some sulfite of calcium or magnesium or both is desired, calcium hydroxide or magnesium hydroxide or both may be suspended in water and 60 utilized in the accumulator to absorb  $\text{SO}_2$ ,

from the steam, thereby forming the sulfite.  $\text{Ca}_2\text{SO}_3$  or  $\text{MgSO}_3$  or mixtures thereof may be further sulfited to form solutions of these in sulfurous acid, or they may be employed to react with sodium carbonate in solution forming sodium sulfite therein and undissolved  $\text{CaCO}_3$  and/or  $\text{MgCO}_3$ . Where such suspensions of hydroxide are thus employed, means should be provided to adequately keep them in suspension and thereby facilitate the 75 step.

It is advantageous to employ some alkaline residual liquor for admixing with acid residual liquor prior to the concentrating step of the cycle. However, it is possible to employ some of the sodium carbonate and relatively high sodium sulfid material or even some of the sodium carbonate and relatively low sodium sulfid material for such treatment of acid residual liquor. Either of these materials will combine with and fix acid constituents of the acid residual liquor and thus aid in the subsequent production of a mixture of sodium carbonate and sodium sulfid. 80

The lime mud which results from the step 90 of treating a solution of sodium carbonate containing sodium sulfid with lime to produce the alkaline cooking liquor, usually contains some calcium hydroxide. When such product has been suitably washed to free it 95 from objectionable amounts of sodium sulfid, some of this washed lime mud may be employed to assist in clarifying the sodium carbonate liquor which is free from or contains but a relatively small amount of sodium sulfid. Such sodium hydroxide as may result 100 from such treatment is present in the liquor which is to be sulfited, and liquor so produced is usually substantially free from iron compounds. Any required oxidizing treatment to 105 advantageously alter sulfur compounds therein may be conducted prior to such clarification step, especially when the lime mud so employed is free from objectionable compounds, or it may be employed coincident with such treatment with the lime mud, or even subsequent thereto, depending upon the 110 circumstances and the requirements, so long as the liquor which is being sulfited is of the required composition so that suitable acid sulfite liquor may be readily produced therefrom. 115

We claim:

1. In a cyclic process for producing chemical pulp, the steps which include cooking one 120 lot of wood in a cooking liquor which contains sulfurous acid and sodium bisulfite, thereby producing one type of residual liquor, cooking another lot of wood in a cooking liquor which contains sodium hydroxide and a lesser amount of sodium sulfid, thereby 125 producing another type of residual liquor, mixing residual liquor of the one type with residual liquor of the other type, separating suspended matter therefrom, adding a regu- 130

lated amount of sodium compound capable of redissolving remaining suspended organic material, concentrating the resulting liquor to produce a concentrated liquor, subjecting 5 constituents of one portion of the concentrated liquor to a reducing furnace treatment to form a product containing sodium carbonate and a considerable amount of sodium sulfid, subjecting constituents of another portion 10 of the concentrated liquor to a furnace treatment to form a product containing the soda mainly as sodium carbonate and free from any considerable amount of sodium sulfid, forming separate liquors 15 from soda compounds in each of the respective products, subjecting the liquor which contains the greater proportion of sodium sulfid to a causticing treatment to form a cooking liquor which contains sodium hydroxide and sodium sulfid, subjecting the other liquor to a regulated treatment to 20 form a cooking liquor containing sodium bisulfite and sulfurous acid and being free from an objectionable amount of sodium 25 thiosulfate.

2. In claim 1, the regulated treatment for obtaining the acid sulfite cooking liquor including the step of oxidizing any sodium sulfid and any sodium thiosulfate in the 30 liquor prior to the sulfiting step.

3. In claim 1, the further step which comprises adding the separated organic material to concentrated liquor produced by the concentrating step.

35 4. In claim 1, the further step which includes feeding one portion of the concentrated liquor into a disc-evaporator and subsequently subjecting constituents thereof to a reducing furnace treatment.

40 5. In claim 1, the further step which comprises mixing gases from the furnaces and employing the mixture for the generation of steam by passing it through a boiler.

45 6. In claim 1, the further step which comprises subjecting the furnace gases to an electrical precipitation treatment to remove solids therefrom.

50 7. In claim 1, the further improvement characterized by subjecting the furnace gases to an electrical precipitation treatment at a temperature above the dew point.

55 8. In claim 1, the further improvement which includes subjecting the furnace gases to an electrical precipitation, recovering the precipitated solids and adding them to the constituents which are to be subjected to a reducing furnace treatment.

60 9. In claim 1, the further step which includes absorbing an oxide of sulfur from furnace gases and employing such compound in a cooking operation of the cycle.

65 10. In claim 1, the improvement which includes absorbing sulfur dioxide from furnace gases in an alkaline soda liquor, and em-

ploying the sodium sulfite thus formed in the acid sulfite type of digestion of the cycle.

11. In claim 1, the further improvement which includes employing the sulfite radicle from the furnace gases so as to sulfite sodium carbonate contained in the liquor which is substantially free from sodium sulfid. 70

12. In claim 1, the further step which comprises relieving steam and sulfur dioxide from acid liquor contained within a digester and absorbing the sulfur dioxide in a soda-containing liquor contained within a vessel of the closed type. 75

13. In claim 1, the further improvement which comprises relieving steam and sulfur dioxide from acid liquor contained within a digester and absorbing the sulfur dioxide in a soda-containing liquor contained within a vessel of the closed type, removing the resulting steam from the vessel and employing it in heating one of the liquors of the cyclic operation. 80

14. In claim 1, the further improvement which comprises relieving steam and sulfur dioxide from acid liquor contained within a digester and absorbing the sulfur dioxide in a soda-containing liquor within a vessel of the closed type, further sulfiting the liquor after removal from the vessel and employing the same in the acid cooking step of the cycle. 85

15. In claim 1, the further improvement which comprises relieving the steam and sulfur dioxide from acid liquor contained within a digester, absorbing some of the relieved steam and sulfur dioxide in liquor contained within another digester to increase the amount of uncombined sulfurous acid therein. 90

16. In claim 1, the further improvement which comprises producing an adequate amount of residual liquor of the alkaline type to serve for neutralizing the acid ingredients of the residual liquor of the acid type and to serve for producing the soda product which contains mainly sodium carbonate and little or no sodium sulfid which is to be sulfited to produce the cooking liquor of the acid type. 100

17. In a process for producing pulp which includes cooking wood by an acid sulfite cooking liquor, the steps which include relieving sulfur dioxide and steam from the digester, absorbing the SO<sub>2</sub> in a liquor containing a reactive alkaline compound whereby a sulfite is formed, further sulfiting the liquor to form the required amount and ratio of combined to uncombined SO<sub>2</sub>, and employing the steam for heating liquor employed in the process. 115

18. A cyclic process for producing chemical pulp which comprises cooking one lot of wood in a cooking liquor which contains sulfurous acid and sodium bisulfite, thereby producing one type of residual liquor, cooking another lot of wood in a liquor which contains sodium hydroxide and a lesser amount 120

125

- of sodium sulfide, thereby producing another type of residual liquor, mixing residual liquor of the one type with residual liquor of the other type, separating suspended matter therefrom, adding a regulated amount of sodium compound capable of redissolving remaining suspended organic matter, concentrating resulting liquor to produce a concentrated liquor, subjecting constituents of one portion of the concentrated liquor to a reducing furnace treatment to form a product containing sodium carbonate and a considerable amount of sodium sulfide, subjecting the constituents of another portion of the concentrated liquor to a furnace treatment to form a product containing the soda mainly as sodium carbonate and free from any considerable amount of sodium sulfide, forming separate liquors from the soda compounds of each of the respective products, subjecting the liquor which contains the greater proportion of sodium sulfide to a causticizing treatment to form a cooking liquor which contains sodium hydroxide and sodium sulfide, subjecting the other liquor to a regulated treatment to form a cooking liquor containing sodium bisulfite and sulfurous acid free from an objectionable amount of sodium thio-sulfate, mixing gases from the furnace, supplying a regulated amount of air to burn combustible material of said gases and employing the hot mixture of gases for the generation of steam by passing it thru a boiler.
19. The cyclic process of producing pulp which comprises cooking one lot of wood in an acid liquor which contains sodium bisulfite, thereby producing one type of residual liquor, cooking another lot of wood in a cooking liquor which contains sodium hydroxide and a lesser amount of sodium sulfide, thereby producing another type of residual liquor mixing residual liquor of the first type with a portion of the residual liquor of the second type, treating the mixture of liquor so formed to produce a white liquor suitable for use in the second named cooking treatment, utilizing another portion of the second type of residual liquor in a preliminary partial cooking treatment, separating residual liquor from the partially cooked wood, treating the last named residual liquor to recover its sodium content, principally as sodium carbonate free from objectionable amounts of sodium sulfide, and treating this soda product to produce an acid cooking liquor.
20. The cyclic process as defined in claim 19 in which white liquor is added to the partially cooked wood and adhering residual liquor and the cooking process completed therewith.
21. The cyclic process according to claim 19 in which the acid liquor is utilized in the first named cooking process.
22. The cyclic process according to claim 19 in which the white liquor is utilized to complete the production of pulp from the partially cooked wood and the acid liquor is utilized for cooking further amounts of wood according to the first named cooking process, and the acid cooking liquor and the alkaline cooking liquor are used in such proportion that the residual liquor of the second type will be sufficient in amount to neutralize the residual liquor of the first type and also to supply sodium compounds sufficient to regenerate the necessary amount of acid cooking liquor.
23. The cyclic process for producing pulp which comprises cooking one lot of wood in a cooking liquor of one type, cooking another lot of wood in a cooking liquor of a different type, separating residual liquors from the pulp resulting from each cooking treatment, mixing said residual liquors, furnacing the solid constituents of the mixture, recovering the valuable constituents of the resulting furnace product, treating a portion of said constituents to regenerate a cooking liquor of the first type and treating another portion of said constituents to regenerate a liquor of the second type.
24. The cyclic process for producing pulp which comprises cooking one lot of wood in an acid cooking liquor, cooking another lot of wood in an alkaline cooking liquor, separating residual liquors from the pulp produced in each cooking treatment, mixing the residual liquors so as to substantially neutralize each of them and precipitate organic matter therefrom, separating the precipitated organic matter, concentrating the residual liquor, subjecting the concentrated liquor to a suitable furnacing operation, recovering valuable constituents from the resulting furnace product, treating a portion of the said constituents to produce an acid cooking liquor suitable for the first named cooking process and treating another portion of said constituents to produce an alkaline cooking liquor suitable for the second named cooking treatment.
25. The cyclic process for producing pulp which comprises cooking one lot of wood in a cooking liquor which contains a sulfite of sodium, cooking another lot of wood in a cooking liquor which contains sodium hydroxide, separating residual liquors from the pulp resulting from each cooking treatment, mixing said residual liquors, subjecting solid constituents of said mixture to a furnacing treatment, recovering sodium compounds from the resulting furnace product, treating a portion of said sodium compounds to produce a sulfite liquor adapted for use in the first named cooking treatment, and treating another portion of the sodium compounds to produce a caustic liquor suitable for use in the second named cooking treatment.
26. The process according to claim 25 in which the furnacing treatment is maintained

under reducing conditions, the portion of the sodium compounds which is to be used for producing a sulfite liquor is subjected to a regulated oxidizing treatment until substantially all the sodium sulfide contained therein has been oxidized.

27. A cyclic process for producing pulp which comprises cooking one lot of wood in a cooking liquor which contains sodium bisulfite, cooking another lot of wood in a cooking liquor which contains sodium hydroxide and sodium sulfide, separating residual liquors from the pulp resulting from each cooking treatment, mixing said residual liquors whereby organic matter is precipitated therefrom, separating organic matter, concentrating the resultant liquor, subjecting solid constituents of the liquor to a furnacing treatment under reducing conditions, leaching the resulting furnace product to produce a solution which contains sodium carbonate and sodium sulfide, subjecting a portion of said solution to a regulated oxidizing treatment until substantially all the sodium sulfide has been oxidized, sulfiting the resulting solution to produce a cooking liquor suitable for use in the first named cooking treatment, causticizing another portion of the solution containing sodium carbonate and sodium sulfide, and returning the causticized solution for use in the second named cooking treatment.

28. The process according to claim 27 in which the regulated oxidizing treatment comprises adding to the solution an oxidizing sodium salt.

29. The process according to claim 27 in which the regulated oxidizing treatment comprises adding to the solution sodium peroxide.

30. The cyclic process for producing pulp which comprises digesting fibrous material with an acid cooking liquor containing an active sodium compound, digesting fibrous material in a cooking liquor containing alkaline sodium compounds, mixing residual liquor from the acid digestion with residual liquor from the alkaline digestion in amount sufficient to form a substantially neutral mixture, thereby precipitating organic matter, evaporating the mixture, subjecting a portion of the evaporated mixture to a reducing furnacing treatment and the furnace product to a treatment adapted to regenerate a cooking liquor of the second type above mentioned, subjecting another portion to an oxidizing furnacing treatment and the furnace product to a treatment adapted to regenerate a cooking liquor of the first mentioned type, and repeating the process.

In testimony whereof we affix our signatures.

LINN BRADLEY.  
EDWARD P. MCKEEFE.